

## UNITED STATES PATENT OFFICE

2,406,564

## COMPOUNDED LUBRICATING OIL

Dilworth T. Rogers, Plainfield, and John G. McNab, Cranford, N. J., assignors to Standard Oil Development Company, a corporation of Delaware

No Drawing. Application May 10, 1943,  
Serial No. 486,428

25 Claims. (Cl. 252—42.7)

1

This invention relates to lubricants and methods of preparing the same, and more particularly to mineral lubricating oil compositions for use as crank case lubricants for internal combustion engines and to addition agents suitable for retarding the normal deterioration of such oils and for improving other properties of the same. It also relates to materials which may be used generally for inhibiting normal oxidation and deterioration of organic materials.

It is known that the addition of certain types of metal organic compounds to lubricating oils improves various properties thereof, such as their oiliness characteristics and their performance in engines, particularly manifested in the maintenance of a clean engine condition during operation. Various metal compounds which have been used for such purposes include the metal derivatives of such organic compounds as fatty acids, naphthenic acids, alcohols, phenols, and ketones. However, these various metal compounds generally have the disadvantage of tending to corrode alloy bearings, such as the cadmium-silver and copper-lead bearings now so widely used in automotive engines; and this is especially true in engines which operate at relatively high speeds and high temperatures. It is an object of the present invention to provide a new class of addition agents for oils which are to be used as crank case lubricants for internal combustion engines and which exhibit the desirable properties of promoting general engine cleanliness, reducing ring sticking, piston skirt varnish formation and the like, and which not only do not exhibit the corrosion promoting tendencies characteristic of many of the above metal compounds, but also inhibit the corrosiveness of oils to which they are added.

The new class of products which have been found in accordance with the present invention to be highly satisfactory as addition agents for lubricating oils and to be readily obtainable are the products obtained by the reaction of elemental sulfur with certain metal phenates and thiophenates, more specifically, the calcium, barium, strontium, magnesium, and zinc phenates and the corresponding thiophenates containing as substituents in the aromatic nucleus one or more alkyl groups having a total of at least five carbon atoms. It has been found that such reaction products are unusually satisfactory in maintaining engine cleanliness, in inhibiting bearing corrosion, in being stable in the presence of water and in being adapted to use with a wide variety of lubricating oil base stocks.

2

Furthermore, these products can be prepared with relatively little expense and without the use of costly solvents or equipment. Sulfur-containing materials which require sulfur halides for their manufacture must usually be prepared in special corrosion resistant vessels whereas those of the present invention, using only elemental sulfur, do not require special equipment and can even be made in ordinary grease kettles.

10 The new sulfur-containing compositions herein described are also useful as anti-oxidants and for other purposes when incorporated in organic materials other than lubricating oils, as will be more fully explained hereinafter, and in many 15 cases it is not necessary to have alkyl groups present to impart sufficient solubility. The invention includes the reaction products of sulfur with compounds analogous to the phenates and thiophenates, but containing selenium and tellurium in place of oxygen or sulfur, and with 20 compounds in which aromatic nuclei other than benzene nuclei are present.

The invention includes the reaction products of sulfur with not only the normal phenates and 25 thiophenates and the like, but the basic metal phenates and thiophenates as well. In a normal phenate of a divalent metal the ratio of metal to phenol is 1 to 2, as in the following formula:

30



35 In a basic metal phenate the ratio of metal to phenol may be 2 to 2 or even 3 to 2. In the case of a 2 to 2 ratio the formula may be

40



45 These basic phenates are formed, for example, by reacting phenols with more than the amount of metallic oxide or hydroxide necessary to form the normal phenates.

We are aware that the metal salts of alkyl 50 phenol sulfides have already been proposed as detergent additives for crankcase lubricants and have indeed been found to be quite effective for this purpose. These materials are usually prepared by the reaction of alkylated phenols with 55 halides of sulfur to give alkylated phenol thio-

ethers or disulfides which are then converted to metal salts by appropriate means. Such products have the general structure



in which the sulfur is present as a bridge linking the aryl groups. In the above formula M is a metal, R is an alkyl substituent and n is a small integer, usually 1 or 2.

The products of the present invention however, which are prepared by first converting alkyl phenols to their metal salts and then causing the salts to react with elemental sulfur, are of an entirely different structure. Although the exact structure of these products is not fully understood, it is certain that the compounds do not contain a sulfur bridge between aryl nuclei as is the case with the metal salts of phenol sulfides, and it is probable that the sulfur is attached directly to the metal through secondary valence forces, as in the following formula:



which probably represents a product formed when two atomic proportions of sulfur are reacted with one molecular proportion of barium tert.-octyl phenate.

One basis for believing that the sulfur is attached to metal rather than to carbon is that during the reaction of metal phenate with sulfur there is no evolution of hydrogen sulfide. Another is that when the product is treated with hydrochloric acid it breaks down to an alkylated phenol, losing both metal and sulfur. On the other hand, similar treatment of a metal alkyl phenol sulfide with hydrochloric acid causes loss of metal only and the final product is the alkylated phenol sulfide.

As has already been pointed out, it is intended that the present invention include products of reaction of sulfur not only with normal metal phenates but also with the basic metal phenates where the ratio of metal to phenol is greater than 1 to 2 and may be as high as 3 to 2. Such products are very easily obtained and are believed to have the same type of structure as those from the normal metal phenates, i. e., the sulfur is attached directly to the metal.

The new class of addition agents employed in accordance with the present invention may be defined in its broadest scope as the reaction products of elemental sulfur with a compound having the formula—

ArXMT

In this formula Ar is an aromatic nucleus and may, for illustration, be a benzene nucleus, or it may consist of a plurality of rings, as in biphenyl, or it may be a condensed nucleus, exemplified by naphthalene, anthracene and the like. X in the formula is a non-metal of group VI of the periodic table. M is a divalent metal of group II of the periodic table, the most important being calcium, barium, strontium, magnesium and zinc,

although for some purposes corresponding compounds containing tin, lead, cobalt or nickel will also be found to be desirable. T in the formula represents either a hydroxyl group or the group—

$(OM)_nXAr$

where M, X, and Ar have the meanings given above and n is 0, 1 or 2. Compounds particularly suited for the purposes of the present invention are formed by reacting sulfur with a compound of the formula—

$(RARX)_nM$

where R represents at least one alkyl radical attached to the nucleus, the total number of carbon atoms in all of such alkyl radicals being at least 5 when the compound is to be dissolved in hydrocarbon oils, other symbols having the meanings given above. It should be understood that the above general formulas include compounds in which various substituent atoms or groups may be attached to the aromatic nucleus, such as alkyl groups, aryl groups, carboxyl groups, hydroxyl groups, alkoxy groups, sulfhydryl groups, halogen atoms, metal substituted carboxyl groups, metal substituted hydroxyl groups, metal substituted sulfhydryl groups, etc. Alkyl radicals attached to the nucleus will preferably have a total of 5 to 12 carbon atoms in all of such groups, but in some cases there may be as many as 16 to 20 carbon atoms in a single group or a plurality of groups. If more than one alkyl group is present in a single molecule, whether or not attached to the same aryl nucleus, such groups may be alike or different. Also included within the class of metal derivatives defined above are the metal salts of phenol sulfides and alkylated phenol sulfides.

Some of the more preferred products to be used in accordance with the present invention are the products to be obtained by reacting sulfur with the following compounds:

Barium tertiary octyl phenate  
Barium di-(tertiary octyl) phenate  
Calcium tertiary octyl phenate  
Barium di-(tertiary amyl) phenate  
Barium cetyl phenate  
Zinc isohexadecyl phenate  
Calcium salt of petroleum phenols  
Barium salt of wax-alkylated phenol  
Magnesium salt of octadecyl cresol  
Barium salt of phenol alkylated with refinery olefin polymers  
Barium salt of tertiary octyl phenol sulfide

Suitable alkylated phenols for use in the present invention may be prepared by alkylating phenol, cresol, naphthol or other phenolic compounds with such alkylating agents as alcohols, alkyl halides, alkyl phosphates, olefins, and the like, with the aid of catalysts such as aluminum chloride, boron fluoride and other metal halides, hydrochloric acid, hydrofluoric acid, sulfuric acid, phosphoric acid, activated clay, etc. Conveniently, olefinic material such as petroleum refinery gases, containing mixtures of olefins, may be used, or preferably individual olefins may be employed, such as butene, amylene or an olefin polymer, such as di-isobutylene or tri-isobutylene. High molecular weight alkylated phenols may also be used, for example, those prepared by condensing phenols with chlorinated paraffin wax, chlorinated petrolatum, or with a chlorinated kerosene or gas oil. Naturally occurring phenols, such as those obtained by alkaline extraction of certain

petroleum stocks or those obtained from cashew nut shell liquid or from other vegetable sources may likewise be used. Halogenated or nitrated phenols will also find application in this invention, particularly if the final additive is to be employed in extreme pressure lubricants.

One class of alkyl phenols which are particularly preferred are those which have been prepared by alkylation of phenol with an olefin polymer such as diisobutylene or a refinery butene polymer oil. Alkylation of phenol with about an equimolecular proportion of diisobutylene gives para-tert.-octyl phenol, also known as diisobutyl phenol or tetramethyl butyl phenol. This phenolic material is especially desirable because of its ease of synthesis and because products made from it are highly satisfactory for the present invention. In many instances, however, a higher degree of alkylation may be advantageous and for this reason the phenol may be alkylated with as much as two molecular equivalents of diisobutylene to give, under proper conditions, essentially di-tert.-octyl phenol, or it may be alkylated with other olefin polymers such as triisobutylene, other isobutylene polymers, or a normal butene polymer. It should be understood that in many cases the alkylation products may be mixtures of various compounds rather than entirely one specific alkyl phenol and that such mixtures may be used in practicing this invention.

For converting the phenolic materials to metal phenates any convenient and effective means may be employed. For example, sodium or potassium salts may first be formed by reaction with sodium or potassium hydroxide and those salts then converted to the desired divalent metal salts by double decomposition. Another method which may be used is the reaction of an alcoholate of the desired metal with the alkylated phenol. When it is possible, the most convenient method is to react the alkylated phenol directly with the oxide or hydroxide of the desired metal. Thus, the barium salts can be prepared directly by adding barium hydroxide to a mineral oil solution of the alkyl phenol at an elevated temperature.

By employing more than the theoretically required amount of divalent metal hydroxide or oxide in the neutralization, it is possible to prepare basic metal salts of the alkylated phenols, that is, salts in which one valence of the polyvalent metal is satisfied by a hydroxyl group. Reaction products of sulfur with basic metal alkyl phenates are particularly useful in extreme pressure lubricants and are also advantageous in motor oils prepared from naphthenic base stocks.

When reacting sulfur with a metal phenate it is usually preferable to use from 2 to 3 atomic proportions of sulfur for each atomic proportion of metal, since in general this range imparts optimum corrosion inhibiting properties to the product. If too large a proportion of sulfur is used, oils containing the resultant additives tend to stain copper or alloys containing the same. The best results are usually obtained when about 2.5 atomic proportions of sulfur are added for each atomic proportion of metal.

Although these proportions are generally preferred for the preparation of crankcase oil additives, lower or higher percentages of sulfur may be employed when the additives are to be used as antioxidants for other organic materials, and as addition agents for extreme pressure lubricants.

If desired, the products used in accordance with this invention may be prepared by the simul-

taneous reaction of an alkylated phenol, a polyvalent metal oxide or hydroxide and elemental sulfur. However, in order to avoid the formation of oil-insoluble materials, it is preferred to first form the metal phenate and then react this with sulfur. Also, although the reaction can be brought about by fusing the reactants together, it is more convenient to carry out the reaction with the aid of solvents, particularly high boiling hydrocarbon solvents, such as xylol or a petroleum fraction. A particularly preferred reaction medium is a lubricating oil fraction, since the final reaction product can thus be obtained as a mineral oil concentrate of the desired additive. Such concentrates may be conveniently stored or shipped as such to save weight and space and may later be readily blended with a lubricating oil base stock in the desired concentration to form a finished lubricating oil blend.

Other preferred classes of products useful in accordance with this invention are those obtained by the reaction of free sulfur with metal salts of alkylated phenol sulfides and with metal phenate salts of alkylated hydroxy carboxylic acids and their carboxylate salts, for example, the barium salt of tertiaryoctyl phenol sulfide and the barium phenate-zinc carboxylate of lauryl salicylic acid.

It is likewise often practical to apply this reaction with free sulfur to other organic compounds containing the —OM group, such as the metal alcoholates or the metal ketonates; for example, calcium octadecylate, barium salts of wax alcohols, etc., to form compositions useful as lubricating oil additives.

The additives may generally be prepared by first dissolving an alkylated phenol in a mineral oil or other suitable solvent and treating the same with a metal hydroxide, e. g., Ba(OH)<sub>2</sub>·8H<sub>2</sub>O, at 90° to 210° C. After a further period of heating, free sulfur is added, whereupon almost instantaneous reaction occurs, the solution assuming a deep red color and becoming more fluid. After additional heating the product is filtered, giving a concentrate of the desired additive. If a calcium salt is to be prepared, a less direct reaction is preferred, since the reaction of alkylated phenols with calcium oxide or hydroxide does not proceed as readily as in the case of barium compounds. Calcium alkyl phenates are preferably prepared by reacting alkyl phenols with calcium methylate or other calcium alcoholate. As to temperatures, the alkylated phenol may be reacted with a metal hydroxide or alcoholate at 90° to 210° C., preferably at 150° to 190° C. Subsequent sulfurization may also be carried out at 90° to 210° C., preferably at 170° to 190° C. It has been found that products prepared by sulfurizing at 180° to 190° C. are the most desirable from the standpoint of water resistivity and freedom from the tendency to stain copper.

It has been found, when preparing these additives in mineral oil, that good results are obtained if a minor proportion of a higher alcohol, such as lauryl, cetyl, stearyl, wool fat alcohol and the like, is added to the reaction mixture in which the compounds of the present invention are prepared. It has been determined by test that substantially none of the higher alcohol enters into the reaction. This alcohol reduces foaming during the process and acts as an auxiliary solvent for the final additive. The best results are obtained by adding a sufficient quantity of the alcohol to give a concentration of about 3% to 15% in the final additive concentrate.

Generally, the additives of the present invention

are most advantageously blended with lubricating oil base stocks in concentrations between the approximate limits of 0.02% and 5.0% and preferably from 0.1% to 2.0%, although larger amounts may be used for some purposes. The exact amount of addition agent required for maximum improvement depends to a certain extent on the particular products used, the nature of the lubricating oil base stock and the general operating conditions of the engine in which the lubricant is to be employed. This same general range of concentration will also be effective when the additives are to be used in greases and in extreme pressure lubricants, although in the latter instance greater amounts may also be employed.

As has been pointed out elsewhere in this specification, it is often convenient to prepare concentrates of the additives in oil, containing, say, 25 to 75% of effective addition agent, the concentrate later being added to a suitable lubricating oil base stock to give a finished blend containing the desired percentage of additive. Thus, when using a 40% concentrate, 2.5% of this material will be blended with a suitable base stock to give a finished oil containing 1% of effective addition agent.

It has also been found that products of better oil solubility can sometimes be obtained when sulfurizing in the presence of small proportions of olefinic material, such as tetraisobutylene, cracked gas or an unsaturated alcohol.

In the following examples are described various preparations of products in accordance with this invention and the results obtained on testing the same in various lubricating oil blends. It is to be understood that these examples, given for illustrative purposes only, do not limit the scope of the invention in any way.

#### EXAMPLE 1

618 parts by weight of p-tert.-octyl phenol (prepared by reacting diisobutylene with phenol in the presence of  $\text{SnCl}_4$  and  $\text{HCl}$  as catalysts at 20° to 85° C.) and 225 parts by weight of commercial stearyl alcohol are added to 1125 parts by weight of mineral oil (a solvent extracted Mid-Continent paraffinic oil of 52 seconds viscosity (Saybolt) at 210° F.). The temperature is raised to 180° C. and the solution agitated and maintained at this temperature while 450 parts by weight of barium hydrate ( $\text{Ba(OH)}_2 \cdot 8\text{H}_2\text{O}$ ) are added gradually. The temperature is held at 180° C. for a period of one hour after the addition of the barium hydrate is completed and then lowered to 170° C. 70 parts by weight of powdered sulfur are added and the temperature is raised to 190° C., and heating is continued until a sample withdrawn from the reaction mixture stains copper only mildly. The mixture is then passed through a filter press yielding a finished product containing 9% barium and 3.3% sulfur.

For some purposes it is often desirable in such reactions to add slightly less than one molecular proportion of barium hydrate for each two molecular proportions of alkyl phenol in order to avoid the formation of basic barium phenates. When crude p-tert.-octyl phenol containing  $\text{HCl}$  and  $\text{SnCl}_4$  catalyst is used, it should be washed with water to remove the  $\text{HCl}$ . All of the barium hydrate should be added to the phenol solution before the sulfur is introduced to avoid the formation of oil-insoluble products.

#### EXAMPLE 2

618 parts by weight of p-tert.-octyl phenol (prepared as in Example 1) and 225 parts of com-

mercial stearyl alcohol were added to 1125 parts by weight of a refined mineral lubricating oil of about 52 seconds viscosity (Saybolt) at 210° F., and the mixture heated to 100° C. Over a period of one hour 465 parts of  $\text{Ba(OH)}_2 \cdot 8\text{H}_2\text{O}$  were added and the mixture was then heated to 170° C. for an additional hour. The temperature was lowered to 120° C., 115 parts of sulfur were added and the temperature raised to 210° C. for a 45-minute period, after which the reaction mixture was filtered, yielding an additive concentrate containing 9.10% barium and 5.06% sulfur.

#### 8

15 A mixture of 618 parts of p-tert.-octyl phenol (prepared as in Example 1), 225 parts of commercial stearyl alcohol and 1125 parts of refined mineral lubricating oil of S. A. E. 20 grade were added at 140° to 150° C. and to this were added 20 465 parts of  $\text{Ba(OH)}_2 \cdot 8\text{H}_2\text{O}$  over a period of one hour. Heating was continued at 150° to 180° C. for an additional hour, the temperature lowered to 150° C. and 70 parts of sulfur were added. Heating was continued for 45 minutes at 150° to 25 170° C. and the product was then filtered. The resulting additive concentrate was a clear red solution which was found to contain 8.88% barium and 3.35% sulfur.

#### EXAMPLE 4

30 This preparation is similar to that described in Example 3, except that larger quantities of materials were used and the preparation was carried out in an ordinary laboratory grease kettle. A mixture of 1854 parts by weight of p-tert.-octyl phenol (prepared as in Example 1), 675 parts of commercial stearyl alcohol and 3370 parts of refined mineral lubricating oil of 52 seconds viscosity (Saybolt) at 210° F. was heated to 35 150° C. Over a 1 1/2 hour period 1350 parts of  $\text{Ba(OH)}_2 \cdot 8\text{H}_2\text{O}$  were added, after which the temperature was raised to 175° C. and held at this point for one hour. The mixture was cooled to 40 150° C., 210 parts of sulfur added, and the temperature raised to 195° C. and maintained at 45 this point for one hour. The product was filtered and the filtered material was found to contain 8.86% barium, and 3.23% sulfur.

#### EXAMPLE 5

50 Over a two-hour period 945 parts by weight of  $\text{Ba(OH)}_2 \cdot 8\text{H}_2\text{O}$  were added to a mixture of 412 parts of p-tert.-octyl phenol (prepared as in Example 1), 203 parts of commercial stearyl alcohol and 1015 parts of a refined paraffinic mineral lubricating oil of S. A. E. 20 grade, the temperature being maintained at 150° C. The temperature was then raised to 180° to 190° C. for one hour, lowered to 150° C. long enough to permit the addition of 128 parts of sulfur and then 55 raised again to 180° to 190° C. for an additional hour. The product was filtered and yielded a dark colored concentrate containing 43% of additive in mineral oil. Analysis showed that the concentrate contained 17.83% barium and 5.79% sulfur.

#### EXAMPLE 6

To 1514 parts by weight of a refined paraffin type mineral lubricating oil of 52 seconds viscosity (Saybolt) at 210° F. were added 702 parts of 2,4-di-tert.-amyl phenol and 304 parts of commercial stearyl alcohol. The mixture was heated to 115° to 120° C. and held at this point while 615 parts of  $\text{Ba(OH)}_2 \cdot 8\text{H}_2\text{O}$  were added over a 70 90-minute period. 105 parts of sulfur were then

added, heating was continued at 120° C. for an additional hour and then the temperature was raised to 150° C. for another hour. The reaction mixture was filtered giving a 40% concentrate of metal-containing additive in mineral oil. Analysis of the concentrate showed 5.82% barium, and 3.38% sulfur.

## EXAMPLE 7

This preparation is similar to that of Example 6 except that no stearyl alcohol was used and the barium compound added was  $\text{Ba(OH)}_2 \cdot \text{H}_2\text{O}$  rather than  $\text{Ba(OH)}_2 \cdot 8\text{H}_2\text{O}$ . 702 parts of 2,4-di-tert.-amyl phenol were added to 1149 parts of a refined paraffinic mineral oil of 52 seconds viscosity (Saybolt) at 210° F. and the mixture heated to 105° C. Then 213 parts of  $\text{Ba(OH)}_2 \cdot \text{H}_2\text{O}$  were added over a period of one hour. During the latter portion of this step about 400 parts by weight of 91% isopropyl alcohol were added in alternate portions with the remainder of the barium hydroxide. The temperature was raised to 120° to 130° C. and held at that temperature for one hour. Then an additional amount of 234 parts of the mineral oil were added together with 17 parts of sulfur and the mixture heated for 1½ hours at 125° C. The reaction product was filtered to obtain the final additive concentrate, which was found to contain 5.59% barium and 2.52% sulfur.

## EXAMPLE 8

A mixture of 412 parts of p-tert.-octyl phenol (prepared as in Example 1), 203 parts of stearyl alcohol and 1015 parts of S. A. E. 20 grade refined mineral lubricating oil was heated to 120° C., and 660 parts of  $\text{Ba(OH)}_2 \cdot 8\text{H}_2\text{O}$  added over a 3-hour period. Then 128 parts of sulfur were added and the temperature held at 120° C. for an additional hour, after which the product was filtered. The additive concentrate obtained was found to contain 12.99% barium and 6.24% sulfur.

## EXAMPLE 9

A solution of 824 parts of p-tert.-octyl phenol in 900 parts of benzene was placed in a reaction vessel equipped with a stirrer and reflux condenser, the latter being fitted with a trap to remove water from the reflux stream. The mixture was heated to its boiling point and over a 1½ hour period 632 parts of  $\text{Ba(OH)}_2 \cdot 8\text{H}_2\text{O}$  were gradually added. Heating and stirring were continued for 8 hours at reflux temperature to remove substantially all of the water of reaction through the water trap. The product in the reaction vessel consisted of a yellowish viscous liquid. This was separated from a small amount of unreacted barium hydroxide and then mixed with 900 parts of xylene. The mixture was heated to 130° C., 64 parts of sulfur were added and heating and stirring continued at 130° C. for 7 hours under reflux. The brown liquid product was filtered while hot and the solvent removed from the filtrate by stripping under reduced pressure. Final traces of water were removed by heating the product in a steam-heated open dish, the final material obtained being an oil-soluble resinous solid containing 21.26% barium and 9.80% sulfur.

## EXAMPLE 10

A solution of 60 parts by weight of metallic calcium in about 2,000 parts of methyl alcohol was mixed with 618 parts of p-tert.-octyl phenol (prepared as in Example 1). The mixture was heated on a steam bath for two hours with vigorous stirring and then evaporated to dryness with the aid

of a stream of nitrogen. The solution was taken up with about 2,700 parts of xylene and heated on a steam bath while a stream of nitrogen was passed through until about two-thirds of the liquid had evaporated. About 800 parts of additional xylene were then added, followed by 52 parts of sulfur, and the mixture was heated under reflux for three hours. A stream of nitrogen was again passed through the solution until about 900 parts of xylene had been removed. The temperature was gradually raised to 130° C. over a three hour period. Following this the solution was filtered and one-half of the solution was mixed with 486 parts of a refined mineral oil of S. A. E. 20 grade and 54 parts of commercial stearyl alcohol. The xylene was then removed under 2 mm. pressure at 110° to 115° C. The resulting product was a 40% solution of the sulfurized calcium p-tert.-octyl phenate in oil. Another portion of the filtrate was evaporated to dryness on the steam bath, giving a yellow resinous solid, which was found to contain 6.81% calcium and 5.48% sulfur.

## EXAMPLE 11

In the production of secondary butyl alcohol from refinery butenes the latter are contacted with 75% to 90% sulfuric acid at 20° to 30° C. to form butyl sulfuric esters which are subsequently hydrolyzed to form the alcohol. During contact with the sulfuric acid some of the butenes polymerize and form what is known as a polymer oil. Since the refinery butene feed stock may contain 40-50% of olefinic material in which, in addition to n-butene, 1 to 2% of butadiene, 1 to 3% of isobutene and 1 to 2% of the dimer and/or trimer of isobutene may be present, the exact nature of the polymer oil obtained is not certain. However, it can reasonably be assumed that it comprises a mixture of polymers and copolymers of these various olefins. For the alkylation of phenol to form products useful for preparing materials of the present invention the butene polymer is steam distilled up to 400° F. and the bottoms, boiling essentially from 400° to 650° F., used as the alkylating material. A mixture of 100 parts of phenol and about 240 parts of the polymer oil fraction is saturated with hydrogen chloride at 80° to 130° F. and 10 parts of aluminum chloride are added over a half hour period with stirring. Stirring is continued for an additional 2½ hours at 120° F. and the product is then stripped of unreacted material by distilling to 270° F. with nitrogen and then up to 400° F. with steam. The desired alkylated phenol remains as the bottoms from this distillation. The product contains alkyl groups having an average of 16 to 20 carbon atoms per molecule.

## EXAMPLE 12

A solution of 280 parts by weight of  $\text{C}_{16-20}$  alkylated phenol (prepared as in Example 11) in 90 parts of commercial stearyl alcohol and 450 parts of a refined mineral lubricating oil of 52 seconds viscosity (Saybolt) at 210° F. was placed in a reaction vessel. The mixture was heated to 150° C. and 120 parts of  $\text{Ba(OH)}_2 \cdot 8\text{H}_2\text{O}$  were added over a period of one hour. Reaction took place readily giving a clear light red solution. The reaction mixture was heated for an additional hour at 170° C. whereupon the color darkened somewhat. It was then cooled to 140° C. and 18.7 parts of sulfur were added. The temperature was held at 140° C. for an additional hour and the mixture then filtered, leaving practically no filter residue. The resulting solution of additive in oil was found to contain 5.59% barium and 2.26% sulfur.

## EXAMPLE 13.

A mixture of 578 parts of  $C_{16-20}$  alkylated phenol (prepared as in Example 11) and 1080 parts of a refined mineral lubricating oil of 52 seconds Saybolt viscosity (210° F.) was heated to 180° C. and 260 parts of  $Ba(OH)_2 \cdot 8H_2O$  added thereto. The reaction product was cooled to 150° C. and filtered, yielding a 40% concentrate of the barium alkyl phenate in oil. It contained 6.05% barium.

## EXAMPLE 14

Blends of lubricating oils containing additives prepared in accordance with the present invention were submitted to the standard Indiana oxidation test, described in S. A. E. Journal, vol. 34, 15

5

10

to opposite sides of a stainless steel rod which was then immersed in the oil and rotated at 600 R. P. M., thus providing sufficient agitation of the sample during the test. Air was then blown through the oil at the rate of 2 cu. ft. per hour. To increase the severity of the test, the bearings were washed and weighed at the end of each four hour period and then polished and reweighed before continuing for another four hour period. The results show the cumulative weight loss at the end of each four hour period. The "corrosion life" indicates the number of hours required for the bearings to lose 100 mg. in weight, determined by interpolation or extrapolation of the data obtained. The results are shown in Table II.

Table II

| Oil                                     | Cumulative Cu-Pb bearing weight loss (mg./25 sq. cm. of surface) |         |          |          |          |          | Corrosion life, hours |
|-----------------------------------------|------------------------------------------------------------------|---------|----------|----------|----------|----------|-----------------------|
|                                         | 4 hours                                                          | 8 hours | 12 hours | 16 hours | 20 hours | 24 hours |                       |
|                                         | 5                                                                | 181     | 42       | 66       | 283      | 52       | 6                     |
| Base oil                                | 5                                                                | 181     | 42       | 66       | 283      | 52       | 6                     |
| Base oil + 0.625% product of Example 3  | 12                                                               | 26      | 42       | 66       | 283      | 52       | 18                    |
| Base oil + 0.625% product of Example 5  | 0                                                                | 1       | 12       | 31       | 52       | 52       | 28                    |
| Base oil + 0.625% product of Example 2  | 2                                                                | 12      | 21       | 32       | 39       | 190      | 22                    |
| Base oil + 0.625% product of Example 6  | 2                                                                | 4       | 8        | 9        | 9        | 10       | 23                    |
| Base oil + 0.625% product of Example 12 | 3                                                                | 13      | 18       | 32       | 80       | 378      | 21                    |
| Base oil + 0.625% product of Example 13 | 37                                                               | 88      | 155      | -----    | -----    | -----    | 9                     |

page 167 (1934). The results are shown in Table I. The values given represent the number of milligrams of sludge formed from 10 grams of oil at the end of various periods during which the test was run, and the "Indiana life" represents the number of hours required for 10 grams of oil to form 10 milligrams of sludge. The base oil used in each case was a well refined, solvent extracted paraffinic type mineral lubricating oil of S. A. E. 20 grade. It will be seen that the oxidation life of the oil was materially increased by incorporation of the additives.

Table I

| Oil                                                  | Sludge (mg./10 gms. of oil) |          |          |          | Indiana life, hrs. |
|------------------------------------------------------|-----------------------------|----------|----------|----------|--------------------|
|                                                      | 24 hours                    | 48 hours | 72 hours | 96 hours |                    |
|                                                      | 0                           | 0        | 16       | 55       |                    |
| Base oil                                             | 0                           | 0        | 16       | 55       | 63                 |
| Base oil + 0.625% <sup>1</sup> product of Example 10 | 0                           | 0        | 0        | 30       | 80                 |
| Base oil + 0.625% <sup>1</sup> product of Example 6  | 0                           | 0        | 0        | 35       | 79                 |

<sup>1</sup> Representing 0.25% of metal salt.

## EXAMPLE 15

The purpose of the following test was to determine the corrosion inhibiting effect of adding a small quantity of various products prepared as in preceding examples to a lubricating oil base. The same base oil was used in all cases, this being a well refined solvent extracted paraffinic type mineral lubricating oil of S. A. E. 20 grade.

The tests were conducted as follows: 500 cc. of oil to be tested were placed in a glass oxidation tube (13" long and 2 $\frac{5}{8}$ " diameter) fitted at the bottom with a  $\frac{1}{4}$ " bore air inlet tube perforated to facilitate air distribution. The oxidation tube was then immersed in a heated bath so that the oil temperature was maintained at 325° F. during the test. Two quarter sections of automotive bearings of copper-lead alloy of known weight having a total area of 25 sq. cm. were attached

35

40

50

55

65

70

75

to opposite sides of a stainless steel rod which was then immersed in the oil and rotated at 600 R. P. M., thus providing sufficient agitation of the sample during the test. Air was then blown through the oil at the rate of 2 cu. ft. per hour. To increase the severity of the test, the bearings were washed and weighed at the end of each four hour period and then polished and reweighed before continuing for another four hour period. The results show the cumulative weight loss at the end of each four hour period. The "corrosion life" indicates the number of hours required for the bearings to lose 100 mg. in weight, determined by interpolation or extrapolation of the data obtained. The results are shown in Table II.

## EXAMPLE 16

Carbon black dispersion tests were carried out to measure the comparative effectiveness of various oil-soluble additives as agents for dispersing sludge. In these tests 6% by weight of activated carbon was added to each oil blend and thoroughly dispersed in the oil by stirring with an "egg beater" type mixer for 15 minutes while the temperature of the oil was maintained at 250° F. 250 cc. of each blend was then placed in a 250 cc. graduated cylinder and allowed to settle for 24 hours while the temperature was maintained at 200° F. If an additive is not a disperser the carbon black settles rapidly at this point, leaving clear oil at the top in an hour or two. A very effective disperser will maintain the carbon black in suspension so that no change in the opaque slurry is apparent even after a 24 hour period.

With all but the most potent dispersers stratification generally occurs, with a black layer at the bottom (high concentration of carbon black) and a blue opaque layer on top (reduced carbon black concentration). Cases of this type, known as "blue line" separations, are only detectable in reflected light. The base oil used for each test was a solvent-extracted Mid-Continent oil of 52 Saybolt seconds viscosity at 210° F. Results of the tests are given in Table III and show that the additives of the present invention are very effective dispersing agents, being even better in this respect than other commercially available

additives.

Table III

| Oil                                                         | Vol. supernatant oil after 24 hrs. at 200° F., cc. |
|-------------------------------------------------------------|----------------------------------------------------|
| Base oil                                                    | 140                                                |
| Base oil+2.5% product of Example 2                          | 0                                                  |
| Base oil+2.5% product of Example 8                          | 0                                                  |
| Base oil+2.15% commercial detergent additive A <sup>1</sup> | 2.40                                               |
| Base oil+5.0% commercial detergent additive B <sup>1</sup>  | 140                                                |
| Base oil+1.5% commercial detergent additive C <sup>1</sup>  | 170                                                |

<sup>1</sup> Concentrations used were by volume and were those recommended by the manufacturers.

<sup>2</sup> Blue line separation.

#### EXAMPLE 17

In the following tests, lubricating oil blends containing additives of the present invention were tested in a single cylinder Caterpillar Diesel engine run under high temperature, high load conditions, namely, 18.7 B. H. P. output, 850 R. P. M., 195° F. oil temperature and 140° F. temperature for 60 hour periods. After each test was completed the engine parts were examined and given

prepared with a phenol having a high molecular weight side chain.

#### EXAMPLE 18

- 5 An additive prepared by the method of Example 1 was blended in 2.5% concentration in an S. A. E.-30 grade base oil of Mid-Continent origin and submitted to a high speed full load test of 328 hours duration in a Model 71 4-cylinder 10 General Motors Diesel engine. The conditions of the test were 103 B. H. P. output at 2000 R. P. M. with 180° F. water jacket temperature and 230° F. crankcase temperature. The test results were very satisfactory and were even better than those obtained in a similar 300-hour test on a 2.5% blend of metal alkyl phenol sulfide additive concentrate in the same base. This blend contained 0.5% of barium tert.-octyl phenol sulfide, 0.5% of barium tert.-octyl phenol disulfide and 0.25% of stearyl alcohol. The oil blend in each of the above tests contained 1% of metal detergent compound.

The demerit ratings obtained in these two tests are given in the following table.

Table V

| Oil blend                                                                 | Engine demerit ratings |           |               |        | Cu-Pb connecting rod bearing weight loss, mg./bearing |
|---------------------------------------------------------------------------|------------------------|-----------|---------------|--------|-------------------------------------------------------|
|                                                                           | Overall                | Ring zone | Piston skirts | Sludge |                                                       |
| SAE-30 oil+2.5% of additive concentrate of Example 1 <sup>1</sup>         | 1.24                   | 2.64      | 1.88          | 0.61   | 6                                                     |
| SAE-30 oil+2.5% of metal phenol sulfide additive concentrate <sup>1</sup> | 1.67                   | 2.96      | 2.25          | 1.16   | 6                                                     |

<sup>1</sup> Equals 1% of effective addition agent, since in each case the additive concentrates contained 40% of metal additive.

demerit ratings based on their condition. The individual ratings were weighted according to their relative importance and an overall rating calculated from them. It should be pointed out that the lower the demerit rating the better the engine condition and hence the better the oil performed in the engine. In these tests base oil A was a well refined solvent extracted paraffinic mineral lubricating oil of S. A. E. 20 viscosity grade, and base oil B was a solvent extracted Mid-Continent paraffinic oil of 52 seconds viscosity (Saybolt) at 210° F. Results of these tests are shown in the following table:

Table IV

| Oil                                   | Engine demerits |           |               |            |             |
|---------------------------------------|-----------------|-----------|---------------|------------|-------------|
|                                       | Overall         | Ring zone | Skirt varnish | Oil filter | Rings stuck |
| Base oil A                            | 1.41            | 1.76      | 1.25          | 2.25       | 1           |
| Base oil A+2.5% product of Example 3  | 0.86            | 0.94      | 0             | 1.00       | 0           |
| Base oil A+2.5% product of Example 2  | 0.78            | 0.74      | 0             | 1.25       | 0           |
| Base oil A+2.5% product of Example 4  | 0.82            | 0.75      | 0             | 1.25       | 0           |
| Base oil A+2.5% product of Example 6  | 0.74            | 0.65      | 0.06          | 1.00       | 0           |
| Base oil A+2.5% product of Example 5  | 1.02            | 1.31      | 0             | 1.00       | 0           |
| Base oil A+2.5% product of Example 12 | 0.67            | 0.63      | 0             | 1.25       | 0           |
| Base oil B                            | 1.46            | 1.55      | 1.00          | 2.00       | 1           |
| Base oil B+2.5% product of Example 3  | 0.74            | 0.69      | 0             | 1.25       | 0           |

It will be observed that in each instance the engine condition was much better with the compounded oil than with the base oil, although the degree of improvement was not the same in each case. The greatest increase in engine cleanliness resulted when using the product of Example 12,

40 These results show that the additive of the present invention was more effective in maintaining engine cleanliness than was an equivalent concentration of a metal alkyl phenol sulfide additive which has achieved commercial acceptance.

45 Oil blends of additives of the present invention have also been submitted to 36-hour high temperature Chevrolet engine tests and have given very satisfactory results as regards maintenance of clean engine condition and as regards inhibition of bearing corrosion, copper-lead connecting rod bearings having been used in the engine for the purpose of measuring the latter quality.

#### EXAMPLE 19

50 A refined lubricating oil of S. A. E. 20 grade was tested for load carrying capacity on the Almen testing machine. Likewise an oil blend comprising the above base oil plus 2.5% of the additive prepared as in Example 8 was submitted to the same test. The Almen test is described 55 in the Proceedings of the American Petroleum Institute, 13th Annual Meeting, section III, page 119, published December 1932. The results of these tests were as follows:

Table VI

| Oil                                    | Almen test, weights carried—gradual loading |
|----------------------------------------|---------------------------------------------|
| Base oil                               | 1                                           |
| Base oil+2.5% of additive of Example 8 | 15                                          |

70 The improvement in load carrying ability imparted by the additive will readily be noted.

75 Although in most instances the additives of the

present invention will of themselves impart sufficient improvement to lubricating oils to give very satisfactory results, still greater improvement may often be obtained by employing the addition agents in conjunction with other additives of the detergent type such as metal soaps, metal phenates, metal alcoholates, metal phenol sulfides, metal organophosphates, thiophosphates, phosphites and thiophosphites, metal sulfonates, metal thiocarbamates, metal xanthates and thiocarbonates, and the like.

Thus, for example, the addition agents of our invention may be used in mineral lubricating oil in conjunction with one or more of the following representative materials:

Barium tert.-octyl phenol sulfide  
 Cobalt tert.-amyl phenol sulfide  
 Calcium mahogany sulfonate  
 Tin salt of wax alkylated phenol sulfide  
 Strontium mahogany sulfonate  
 Magnesium cetyl phenate  
 Nickel oleate  
 Aluminum-calcium mixed soap of fatty acid from oxidation of petroleum fractions  
 Calcium isohexadecyl phenol sulfonate  
 Barium octadecylate  
 Calcium dichlorostearate  
 Nickel amyl xanthate  
 Calcium phenyl stearate  
 Nickel dibutyl thiocarbamate  
 Barium dioctyl dithiophosphate  
 Zinc methyl cyclohexyl dithiophosphate  
 Calcium dihexadecyl monothiophosphate  
 Calcium cetyl phosphate  
 Barium mahogany sulfonates  
 Zinc diisopropyl salicylate  
 Aluminum naphthenate  
 Magnesium mahogany sulfonates  
 Calcium double salt of octadecyl phenol sulfonic acid  
 Barium phenate-zinc sulfonate of isohexadecyl phenol sulfonic acid  
 Barium di-tert.-amyl phenol sulfide  
 Calcium phenate-barium carboxylate of octadecyl salicylic acid  
 Tin naphthenate

Particularly advantageous are lubricant compositions in which the additives of the present invention are employed in conjunction with metal salts of petroleum mahogany sulfonic acids. Examples of such compositions include the following:

|                                                   | Per cent |
|---------------------------------------------------|----------|
| (1) Additive concentrate of the present invention | 1.5      |
| Calcium mahogany sulfonate                        | 0.5      |
| Mineral lubricating oil                           | 98       |
| (2) Additive concentrate of the present invention | 2.5      |
| Barium mahogany sulfonate                         | 1.2      |
| Mineral lubricating oil                           | 96.3     |
| (3) Zinc mahogany sulfonate                       | 3.5      |
| Additive concentrate of the present invention     | 2.5      |
| Mineral lubricating oil                           | 94       |

The lubricating oil base stocks used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by conventional methods using acid, alkali and/or

clay or other agents such as aluminum chloride, or they may be extracted oils produced, for example, by solvent extraction with solvents of the type of phenol, sulfur dioxide, furfural, dichloroethyl ether, propane, nitrobenzene, crotonaldehyde, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coal tar fractions and coal tar or shale oil distillates may also be used. Also, for special applications, animal, vegetable or fish oils or their hydrogenated or voltolized products may be employed, either alone or in admixture with mineral oils.

For the best results the base stock chosen should normally be that oil which without the new additives present gives the optimum performance in the service contemplated. However, since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at 210° F. For the lubrication of certain low and medium speed Diesel engines the general practice has often been to use a lubricating oil base stock prepared from naphthenic or aromatic crudes and having a Saybolt viscosity at 210° F. of 45 to 90 seconds and a viscosity index of 0 to 50. However, in certain types of Diesel service, particularly with high speed Diesel engines, and in gasoline engine, including aviation engine service, oils of higher viscosity index are often preferred, for example, up to 75 to 100, or even higher, viscosity index.

In addition to the materials to be added according to the present invention, other agents may also be used, such as dyes, pour depressors, heat thickened fatty oils, sulfurized fatty oils, organo-metallic compounds, metallic or other soaps, sludge dispersers, anti-oxidants, thickeners, viscosity index improvers, oiliness agents, resins, rubber, olefin polymers, voltolized fats, voltolized mineral oils, and/or voltolized waxes and colloidal solids such as graphite or zinc oxide, etc. Solvents and assisting agents, such as esters, ketones, alcohols, aldehydes, halogenated or nitrated compounds, and the like, may also be employed.

Assisting agents which are particularly desirable are the higher alcohols having eight or more carbon atoms and preferably 12 to 20 carbon atoms. The alcohols may be saturated straight and branched chain aliphatic alcohols such as octyl alcohol,  $C_8H_{17}OH$ , lauryl alcohol,  $C_{12}H_{25}OH$ , cetyl alcohol,  $C_{16}H_{33}OH$ , heptadecyl alcohol,  $C_{17}H_{35}OH$ , stearyl alcohol, sometimes referred to as octadecyl alcohol,  $C_{18}H_{37}OH$ , and the like; the corresponding olefinic alcohols such as oleyl alcohol; cyclic alcohols, such as naphthenic alcohols; and aryl substituted alkyl alcohols, for instance, phenyl octyl alcohol, or octadecyl benzyl alcohol or mixtures of these various alcohols, which may

be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from those materials, for some purposes, the wool fat, sperm oil or other natural products rich in alcohols may be used per se. Products prepared synthetically by chemical processes may also be used such as alcohols prepared by the oxidation of petroleum hydrocarbons, e. g., paraffin wax, petrolatum, etc. These assisting agents serve to enhance the detergent and sludge dispersive qualities and aid the solubility of the metal-containing additives and at the same time impart some oiliness properties to the lubricating oil compositions.

In addition to being employed in crankcase lubricants the additives of the present invention may also be used in extreme pressure lubricants, engine flushing oils, industrial oils, process oils, general machinery oils, greases and rust preventive compositions. Also their use in motor fuels, Diesel fuels and kerosene is contemplated. A particular application in this regard is their use in motor fuels containing tetraethyl lead or other anti-knock agents, the additives of the present invention serving not only as anti-oxidants for the fuel, but also as stabilizers for the anti-knock agent itself.

Since these additives exhibit antioxidant properties and are believed also to possess the ability to modify surface activity, they may be employed in asphalts, road oils, waxes, fatty oils of animal or vegetable origin, soaps, and plastics. Similarly, they may be used in natural and synthetic rubber compounding both as vulcanization assistants and as antioxidants, and generally they may be used in any organic materials subject to deterioration by atmospheric oxygen.

The present invention is not to be considered as limited by any of the examples described herein which are given by way of illustration only, but it is to be limited solely by the terms of the appended claims.

We claim:

1. An organic material containing a stabilizing quantity of a reaction product of at least 2 gram atoms sulfur with 1 mol of a compound having the structure—



where Ar is an aromatic nucleus, X is a non-metal of group VI of the periodic table, M is a divalent metal of group II of the periodic table and selected from the class consisting of calcium, barium, strontium, magnesium and zinc, and T is a member of the class consisting of OH and  $(\text{OM})_n\text{XAr}$ , where M, X and Ar have the meanings given above and n is a number of the class consisting of 0, 1, and 2.

2. A hydrocarbon product containing a stabilizing quantity of a reaction product of at least 2 gram atoms of sulfur with 1 mol of a compound of the formula—



where Ar is an aromatic nucleus, R represents at least one alkyl radical joined to said nucleus, all of such radicals having a total of at least 5 carbon atoms, X is a member of the group consisting of oxygen and sulfur, M is a divalent

metal of group II of the periodic table and selected from the class consisting of calcium, barium, strontium, magnesium and zinc, and T is a member of the class consisting of OH and  $(\text{OM})_n\text{XArR}$ , where, M, X, Ar and R have the meanings given above and n is a number of the class consisting of 0, 1 and 2.

3. A mineral lubricating oil containing a stabilizing quantity of a reaction product of 2 to 10 gram atoms of sulfur with 1 mol of a compound of the formula



where Ar is an aromatic nucleus, R represents at least one alkyl radical joined to said nucleus, all of such radicals having a total of at least 5 carbon atoms, X is a member of the group consisting of oxygen and sulfur, and M is a divalent metal of group II of the periodic table and selected from the class consisting of calcium, barium, strontium, magnesium and zinc.

4. A lubricating oil according to claim 3 in which X of the formula represents oxygen.

5. A lubricating oil according to claim 3 in which Ar of the formula represents a benzene nucleus and X of the formula represents oxygen.

6. A mineral lubricating oil containing a stabilizing quantity of a reaction product of sulfur with a metal alkyl phenate, in which the alkyl radicals have a total of at least 5 carbon atoms and in which the metal is a divalent metal of group II of the periodic table and selected from the class consisting of calcium, barium, strontium, magnesium and zinc, such reaction product being obtained by reacting from about 2 to about 3 atomic proportions of sulfur to each atomic proportion of the metal of the metal phenate.

7. A lubricating oil according to claim 6 in which the alkyl radical of the phenate is an octyl radical and in which the metal is an alkaline earth metal.

8. A lubricating oil according to claim 6 in which the alkyl radical of the phenate is a p-tert.-octyl radical.

9. A lubricating oil according to claim 6 in which the metal is barium.

10. A mineral lubricating oil containing a stabilizing quantity of a reaction product of at least 2 gram atoms of sulfur with 1 mol of a product obtained by reacting barium hydroxide with a p-tert.-octyl phenol.

11. A mineral lubricating oil containing a stabilizing quantity of the reaction product of 2 to 3 gram atoms of sulfur with 1 mol of a barium di-(tertiary amyl) phenate.

12. A mineral lubricating oil containing a stabilizing quantity of the reaction product of 2 to 3 gram atoms of sulfur with 1 mol of a barium alkylated phenol in which the alkyl groups contain a total of about 16 to about 20 carbon atoms per molecule.

13. A mineral lubricating oil containing a stabilizing quantity of a product obtained by reacting from about 2 to about 3 atomic proportions of sulfur in a mineral oil with 1 atomic proportion of a metal in the form of a metal salt of an alkylated phenol at 100° to 210° C., the metal of said salt being a divalent metal of group II of the periodic table and selected from the class consisting of calcium, barium, strontium, magnesium and zinc, and the alkyl groups of the phenol having a total of at least 5 carbon atoms.

14. A mineral lubricating oil according to claim 13 in which the additive was obtained by re-

acting the sulfur with the metal salt in the presence of a minor proportion of a higher fatty alcohol.

15. A mineral lubricating oil according to claim 13 in which the metal salt is a barium salt and in which the reaction with sulfur is conducted at a temperature of about 170° to about 190° C.

16. A mineral lubricating oil containing a stabilizing quantity of a product obtained by reacting a tert.-octyl phenol with barium hydroxide and further reacting the product thus obtained with from 2 to 3 atomic proportions of sulfur for each atomic proportion of metal present, in a mineral oil solvent at a temperature of about 170° to about 190° C., and in which a sufficient quantity of stearyl alcohol is present during both reactions to provide for a concentration of about 3% to about 15% in the mineral oil containing the final reaction products before blending with the lubricating oil base.

17. As a composition of matter a sulfur-containing product obtained by reacting at least 2 atomic proportions of elemental sulfur with one molecular proportion of metal phenate in which the metal is a divalent metal of group II of the periodic table and selected from the class consisting of calcium, barium, strontium, magnesium and zinc.

18. As a new composition of matter an oil soluble sulfur-containing product obtained by reacting from about 2 to about 3 atomic proportions of elemental sulfur with 1 molecular proportion of a metal octyl phenate, in which the metal is a divalent metal of group II of the periodic table and selected from the class consisting of calcium, barium, strontium, magnesium and zinc.

19. As a new composition of matter an oil soluble sulfur-containing product obtained by reacting about 2 to about 3 atomic proportions of elemental sulfur with one molecular proportion of the reaction product of barium hydroxide and a tert.-octyl phenol.

20. As a new composition of matter an oil soluble sulfur-containing product obtained by reacting about 2 to 3 atomic proportions of

elemental sulfur with one molecular proportion of barium di-(tertiary amyl) phenate.

21. As a new composition of matter an oil soluble sulfur-containing product obtained by reacting about 2 to 3 atomic proportions of elemental sulfur with one molecular proportion of a barium alkylated phenate in which the alkyl groups contain a total of about 16 to about 20 carbon atoms per molecule.

22. The method of preparing an oil-soluble sulfur-containing product having anti-oxidant properties in the presence of a hydrocarbon oil which comprises reacting from about 2 to about 3 atomic proportions of elemental sulfur with 1 molecular proportion of a metal alkyl phenate in which the metal is a divalent metal of group II of the periodic table and selected from the class consisting of calcium, barium, strontium, magnesium and zinc and in which the alkyl groups contain a total of at least 5 carbon atoms.

23. The method of preparing an oil-soluble sulfur-containing product having anti-oxidant properties in the presence of mineral oil which comprises reacting about 2 to about 3 atomic proportions of elemental sulfur with one molecular proportion of the reaction product of barium hydroxide and p-tert.-octyl phenol at a temperature of 90° C. to 210° C.

24. The method of preparing an oil-soluble sulfur-containing product having anti-oxidant properties in the presence of organic material which comprises reacting barium hydroxide with a tert.-octyl phenol in a mineral oil solution at a temperature of about 90° to about 210° C. and further reacting the product thus obtained, while in the mineral oil solution, with from about 2 to about 3 atomic proportions of elemental sulfur for each atomic proportion of metal present, at a temperature of about 170° to about 190° C.

25. Method according to claim 22 in which a small proportion of a higher fatty alcohol is added to the mineral oil solvent before reacting the phenol with the barium hydroxide.

DILWORTH T. ROGERS.  
JOHN G. McNAB.